

# UNITED STATES PATENT OFFICE.

ISIDOR KITSEE, OF PHILADELPHIA, PENNSYLVANIA.

## PROCESS OF EXTRACTING PRECIOUS METALS FROM ORES.

No. 913,735.

Specification of Letters Patent.

Patented March 2, 1909.

Application filed May 23, 1908. Serial No. 434,583.

*To all whom it may concern:*

Be it known that I, ISIDOR KITSEE, citizen of the United States, residing at Philadelphia, in the county of Philadelphia and

5 State of Pennsylvania, have invented certain new and useful Improvements in Processes of Extracting Precious Metals from Ores, of which the following is a specification.

10 My invention relates to an improvement in the process of extracting precious metals from ores and has more special reference to the extracting of gold from the natural deposit.

15 The process of extracting gold from its ores by means of a solution of cyanid of an alkali, or alkaline earth, is now most generally practiced and it is the aim of my invention to render the process more expeditious 20 and more economical.

In extracting gold from its ore, by means of a solution of cyanid, the presence of an oxidizing agent is necessary and is most generally affected by the action of the air upon 25 the gold. Instead of depending upon this agency alone, I employ the anolyte from an electric apparatus in which a compound containing nitrogen is electrolyzed.

I have made experiments with different compounds and found that the compound known as the nitrate of sodium is well adapted for the purpose and has the advantage of being readily attainable. I prefer this com-

pound also on account of its cheapness, as I found that the same may be used in its 35 crude or impure state.

The apparatus in which the compound, such as a nitrate of sodium, or potassium is electrolyzed, should consist of two compartments; one for the cathode and one for the 40 anode.

I do not intend to use the contents of the positive compartment of such an apparatus, as the solvent—*per se*—but I intend to use the same for the purpose of hastening the 45 solvent action of the cyanid.

Having now described my invention, what I claim as new and desire to secure by Letters Patent is—

1. The process of extracting precious 50 metals from their ores, which consists in subjecting the ores to the dissolving action of a cyanid in the presence of the anolyte of an electric apparatus in which a nitrogen compound has been electrolyzed the anolyte 55 containing an oxid of nitrogen.

2. The process of extracting gold from its ores consisting in subjecting the ores to the dissolving action of a cyanid in the presence of an anolyte carrying an oxid of nitrogen. 60

In testimony whereof I affix my signature in presence of two witnesses.

ISIDOR KITSEE.

Witnesses:

EDITH R. STILLEY,  
MARY C. SMITH.